

March 4, 1941.

**C. ADAMOLI**  
**PROCESS FOR THE MANUFACTURE OF ANHYDROUS**  
**BERYLLIUM FLUORIDE FREE FROM OXIDE**

2,233,465

2 Sheets-Sheet 1

Fig. I.



By Carlo Adamoli, Inventor: X-2  
Stebbins, Blenner & Parnell, Attg's.

March 4, 1941.

C. ADAMOLI

2,233,465

PROCESS FOR THE MANUFACTURE OF ANHYDROUS  
BERYLLIUM FLUORIDE FREE FROM OXIDE

Filed Jan. 7, 1939

2 Sheets-Sheet 2



Inventor:  
Carlo Adamoli,  
By Stelbros, Blenko & Pamplie, attys.

## UNITED STATES PATENT OFFICE

2,233,465

PROCESS FOR THE MANUFACTURE OF  
ANHYDROUS BERYLLIUM FLUORIDE  
FREE FROM OXIDECarlo Adamoli, Milan, Italy, assignor to  
Perosa Corporation, Wilmington, Del., a  
corporation of DelawareApplication January 7, 1939, Serial No. 249,828  
In Italy January 10, 1938

10 Claims. (Cl. 23—38)

Presently only two methods are known for producing, in the laboratory, anhydrous beryllium fluoride which is free from oxide and which corresponds to the formula  $\text{BeF}_2$  (Lebeau, Annales de Chimie et de Physique 1869-4- (7) 484; comptes-rendus Académie des Sciences (Paris) 1898 (126) 1418; Gmelins Handbuch, Beryllium System Numercer 26 p. 105)). These two methods have already received applications in the art which apparently considerably differ from another and one of which consists in causing gaseous hydrofluoric acid to react at a temperature between 500 and 750° C. on beryllium oxide, more particularly in the form of dry hydroxide, according to the reaction  $\text{BeO} + 2 \text{HF} = \text{BeF}_2 + \text{H}_2\text{O}$ , while the other consists in forming double ammonium beryllium fluoride in the dry state through the reaction of acid ammonium fluoride on beryllium oxide or beryllium hydrate, and then in distilling the ammonium fluoride according to the reaction  $\text{Be}(\text{NH}_4)_2\text{F}_4 = \text{BeF}_2 + 2 \text{NH}_4\text{F}$ .

These two different methods are both characterized by means adapted for eliminating the salification water which ordinarily causes the hydrolysis of the beryllium fluoride and determines the formation of the beryllium oxide which is generally contained in the known product which is improperly designated under the name of "beryllium fluoride," while it is, in fact, a basic product of various compositions. Now, while they well permit to avoid the hydrolysis of the beryllium fluoride and to obtain this salt in an anhydrous condition, the said methods offer, again, certain technical disadvantages resulting, in one case, in the difficulty of using the gaseous hydrofluoric acid at a high temperature and of working on masses of a large volume and, in the second case, in the double operation consisting in producing the dry ammonium fluoride for subsequently distilling it while using a quantity of fluorine which is double of that which corresponds to the formation of the  $\text{BeF}_2$  and in the difficulty, which is a consequence therefrom, of recuperating the sublimating ammonium fluoride.

The present invention has for its object to provide a commercial process for making anhydrous beryllium fluoride which is free from oxide, the said process permitting of eliminating the above mentioned difficulties. This process is essentially characterized in that neutral or acid ammonium fluoride is caused to act in vacuum and in the hot state on an oxygenated compound of the beryllium such as the dry beryllium oxide, the dry beryllium hydroxide or the beryllium carbonate, the quantity of ammonium fluoride

which is used being such that it substantially corresponds to that which is theoretically necessary for the sole conversion of the beryllium into beryllium fluoride. When starting, for instance, from beryllium oxide and neutral ammonium fluoride, the reaction which characterizes the process according to the invention may then be written as follows:



the ammonia and the water being eliminated as they are formed by the aspiration of the apparatus which serves to maintain the reactional medium under the vacuum.

In order to insure the complete fluorination of the beryllium, it is advantageous to work with a slight excess of ammonium fluoride of less than 5% of the stoichiometric quantity which is necessary for effectuating the above mentioned reaction, or with the addition of a corresponding quantity of acid ammonium fluoride.

It is also advantageous to effectuate the reaction in two successive steps in different conditions of temperature, the first step being effectuated at a temperature which is preferably less than 100° C. and until the escape of ammonia practically ceases, while the second step begins immediately after the first and is effectuated at a higher temperature, preferably between 200 and 250° C. and preferably in the presence of a current of dry inert gas. It may be expedient, for preventing any possible losses in the apparatus, to introduce a small quantity of dry hydrofluoric acid simultaneously with this dry gas.

The invention provides more particularly a form of execution in a cycle of the above defined process, according to which the intimate mixture of the neutral or acid ammonium fluoride with the oxygenated compound of the beryllium and the reaction between these agents are effectuated in closed heated vessels, while preferably fractionating the heating in two or more steps corresponding to increasing temperatures conditions up to a maximum of 250° C., the ammonia which has been formed in a gaseous condition as well as the water which is present and that which forms during the reaction being removed from the said vessels by means of a suitable vacuum pump, the ammonium fluoride being re-formed from the collected ammonia, as, for instance, by causing the latter to pass into a solution of hydrofluoric acid or, preferably, into an already saturated acid solution of ammonium fluoride, the fresh salt which is formed then precipitating immediately.

It is also possible to only recuperate the ammonia in water.

The above mentioned process can be performed with advantage in an apparatus such as that which is shown by way of non limitative example in the appended drawings, in which Figures 1 and 2 show respectively in a vertical diagrammatical sectional view two parts of the apparatus which join according the lines  $x_1-x_2$ .

- 10 As shown in this example, the apparatus comprises a mixer 1 formed of a sloping cylinder in which rotates a propeller 2 which can be driven by a suitable drive (not shown). In its upper part the mixer is provided with a conduit 3 with a tight closure 3a for the introduction of the charge, and in its lower part it is provided with a conduit 4 which permits of the passage of the material which has been treated into a second mixer 5. This latter is also formed of a sloping cylinder in which a propeller 6 rotates in a contrary direction from that of the propeller 2. At the lower part of the mixer 5 there is provided a discharging device 7 for removing the beryllium fluoride which has been formed. Both mixers 1 and 5 are located in a drying oven 8 with two different temperature conditions, one of 80° C., for instance, for the operation in the mixer 1 and the other of 250° C. for the operation in the mixer 5.
- 20 At suitable places, for instance on the conduits 3 and 4, are connected conduits 9, 9a leading to the inner space of a rotating barrel or drum 10 which contains a solution of hydrofluoric acid arriving by a pipe 11a from a recipient 11 and which, preferably, is saturated with ammonium fluoride but maintained acid for insuring the fluorination of the ammonia which has been removed from the mixer 1, as will be explained hereinafter. The drum 10 is provided with filtering vanes 12 adapted for depositing the crystallized ammonium fluoride into a vat 13 secured on the axial support 10a of the drum.
- 30 The inner space of the drum 10 is connected, on the other hand, by means of a conduit 14, 45 with a drying tower 15 which is connected, by means of a conduit 16, with the suction side of a pump 17 the discharge of which is connected by means of conduits 18, 18a with the mixer 5 for the introduction of a neutral gas into the latter.
- 40 The operation of this apparatus is as follows. 50 100 kg. of beryllium hydrate  $Be(AH)_2$  with 60% of  $BeO$  in a granulated form are introduced, for instance, into the mixer 1 with 178 kg. of neutral ammonium fluoride (which quantity can be, if desired, increased up to 185 kg.) or with 137 kg. of ammonium bifluoride (which quantity can be, if desired, increased up to 143 kg.). The material is heated during a certain time in the mixers 1 and 5 to the above indicated temperatures. 60 The materials which have been introduced into the mixer 1 and which are intimately mixed by the propeller 2 pass progressively into the mixer 5, while the ammonia and the steam which escape under the action of the heating are drawn in by the vacuum pump together with the neutral gas which is introduced into the mixer 5 and are derived by the conduits 9, 9a into the absorption apparatus 10. The ammonia is further removed up to the quantity which must be theoretically obtained. Finally about 112 kg. of beryllium fluoride are removed through the discharging device 7. On the other hand, 178 kg. (or eventually from 178 to 185 kg.) of crystallized ammonium fluoride which has been depositated 70 into the vat 13 by the filtering vanes 12 are re-

moved from the absorption apparatus 10 which contains the mother liquors from the preceding operations. The neutral gas which has been recuperated in the drum 10 is dried in the tower 15 and taken again by the pump 17 whereafter it is 5 re-introduced into the mixer 5.

The process of the present application is a modification of the process described and claimed in my Patent No. 2,173,290, granted September 19, 1939. 10

What I claim is:

1. A process for the manufacture of anhydrous beryllium fluoride free from oxide, which consists in causing a compound of the group consisting of ammonium fluoride and ammonium acid 15 fluoride to act in vacuo and in the hot state on an oxygenated beryllium compound belonging to the group consisting of the oxide, the hydrate and the carbonate of beryllium, in a dry state, the proportion of ammonium fluoride which is used 20 substantially corresponding to that which is theoretically necessary for forming only beryllium fluoride.

2. A process for the manufacture of anhydrous beryllium fluoride free from oxide, which consists in causing neutral ammonium fluoride to act in vacuo and in the hot state on an oxygenated beryllium compound belonging to the group consisting of the oxide, the hydrate and the carbonate of beryllium, in a dry state, the proportion of neutral ammonium fluoride which is used substantially corresponding to that which is theoretically necessary for forming only beryllium fluoride. 25

3. A process for the manufacture of anhydrous beryllium fluoride free from oxide, which consists in causing acid ammonium fluoride to act in vacuo and in the hot state on an oxygenated beryllium compound belonging to the group consisting of the oxide, the hydrate and the carbonate of beryllium, in a dry state, the proportion of acid ammonium fluoride which is used 30 substantially corresponding to that which is theoretically necessary for forming only beryllium fluoride. 40

4. A process for the manufacture of anhydrous beryllium fluoride free from oxide, which consists in causing ammonium fluoride to act in vacuo and in the hot state on an oxygenated beryllium compound belonging to the group consisting of the oxide, the hydrate and the carbonate of beryllium, in a dry state, the proportion of ammonium fluoride which is used not exceeding by more than 5% that which is theoretically necessary for forming only beryllium fluoride. 50

5. A process for the manufacture of anhydrous beryllium fluoride free from oxide, which consists in causing to act in a hot state and in vacuo on an oxygenated beryllium compound belonging to the group consisting of the oxide, the hydrate and the carbonate of beryllium in a dry state, ammonium fluoride in a quantity which substantially corresponds to that which is theoretically necessary for forming only beryllium 60 fluoride, and in removing the ammonia and the water vapour from the reactional medium as they are formed.

6. A process for the manufacture of anhydrous beryllium fluoride free from oxide, which consists in causing to act in a hot state and in vacuo on an oxygenated beryllium compound belonging to the group consisting of the oxide, the hydrate and the carbonate of beryllium in a dry state, ammonium fluoride in a quantity which 70

75

substantially corresponds to that which is theoretically necessary for forming only beryllium fluoride, in introducing a dry inert gas into the reactional medium and in removing from the said 5 reactional medium the ammonia and the water vapour as they are formed simultaneously with the inert gas.

7. A process for the manufacture of anhydrous beryllium fluoride free from oxide, which consists in causing to act in a hot state and in vacuo on an oxygenated beryllium compound belonging to the group consisting of the oxide, the hydrate and the carbonate of beryllium in a dry state, ammonium fluoride in a quantity which 10 substantially corresponds to that which is theoretically necessary for forming only beryllium fluoride, in introducing a dry inert gas into the reactional medium with the addition of a small quantity of dry gaseous hydrofluoric acid and in removing from the said reactional medium the ammonia and the water vapour as they are formed simultaneously with the inert gas.

8. A process for the manufacture of anhydrous beryllium fluoride free from oxide, which consists in mixing an oxygenated beryllium compound belonging to the group consisting of the oxide, the hydrate and the carbonate of beryllium in a dry state and ammonium fluoride in a proportion which substantially corresponds to that 25 which is theoretically necessary for forming only beryllium fluoride, in heating this mixture in vacuo up to a temperature of less than 100° C. until the escape of ammonia practically ceases and then to a temperature between 200 and 250° C., in introducing a dry inert gas into the 30 reactional medium during the second step of the heating, and in removing from the said reactional medium the ammonia and the aqueous vapor as they are formed as well as the inert gas, in causing the removed ammonia to pass into a solution of hydrofluoric acid saturated with ammonium fluoride and collecting the latter in a crystalline form, and returning it to the process to treat a further quantity of oxygenated beryllium compound.

9. A process for the manufacture of anhydrous beryllium fluoride free from oxide, which consists in mixing an oxygenated beryllium compound belonging to the group consisting of the oxide, the hydrate and the carbonate of beryllium in a dry state and ammonium fluoride in a proportion which substantially corresponds to that which is theoretically necessary for forming only beryllium fluoride, in heating this mixture in vacuo up to a temperature of less than 100° C. until the escape of ammonia practically ceases and then to a temperature between 200 and 250° C., in introducing a dry inert gas into the reactional medium during the second step of the heating, and in removing from the said reactional medium the ammonia and the aqueous vapor as they are formed as well as the inert gas, and in causing the removed ammonia to pass into a 15 solution of hydrofluoric acid in order to re-form the ammonium fluoride used in the process.

10. A process for the manufacture of anhydrous beryllium fluoride free from oxide, which consists in mixing an oxygenated beryllium compound belonging to the group consisting of the oxide, the hydrate and the carbonate of beryllium in a dry state and ammonium fluoride in a proportion which substantially corresponds to that which is theoretically necessary for forming only 20 beryllium fluoride, in heating this mixture in vacuo up to a temperature of less than 100° C. until the escape of ammonia practically ceases and then to a temperature between 200 and 250° C., in introducing a dry inert gas into the 25 reactional medium during the second step of the heating, and in removing from the said reactional medium the ammonia and the aqueous vapor as they are formed as well as the inert gas, in causing the removed ammonia to pass into a solution of hydrofluoric acid saturated with ammonium fluoride for re-forming ammonium fluoride and collecting the latter in a crystalline form, and returning it to the process to treat a further quantity of oxygenated beryllium compound.

CARLO ADAMOLI.